

May 15, 1934.

C. W. ALLSHOUSE

1,958,506

PAVEMENT AND METHOD OF MAKING SAME

Filed April 16, 1932



FIG. 1



FIG. 2



FIG. 3.



FIG. 4.

INVENTOR.

Carl W. Allshouse

BY

Fay, Oberlin & Fay

ATTORNEYS.

## UNITED STATES PATENT OFFICE

1,958,506

## PAVEMENT AND METHOD OF MAKING SAME

Carl W. Allshouse, East Cleveland, Ohio

Application April 16, 1932, Serial No. 605,623

5 Claims. (Cl. 94—22)

The present invention, relating as indicated to a pavement and method of making the same, is more particularly directed to a new and improved coated brick pavement and to a method 5 of treating such a pavement, either during its initial construction or subsequently to prevent the excess bitumen employed as a filler between the brick from rendering the pavement dangerously slippery to traffic. The principal object 10 of the invention is the provision of a pavement of the character described and a method of treating the same which shall be simple and economical, and effective to improve materially the traction qualities of the surface.

15 To the accomplishment of the foregoing and related ends, said invention, then, consists of the means hereinafter fully described and particularly pointed out in the claims; the following description and the annexed drawing setting 20 forth in detail one product and one method constituting, however, but one of various applications of the principle of my invention.

In said annexed drawing:

Fig. 1 is a partial transverse section of a brick 25 pavement embodying my improved invention illustrating the application of my method of treating to the same; Fig. 2 is a similar view of the same pavement following treatment; Fig. 3 is a similar view on an enlarged scale; and Fig. 4 is 30 a similar view of an asphaltic covered concrete pavement.

In the ordinary brick pavement bricks are initially laid or set ordinarily upon a sand cushion, which in turn constitutes a coating over a 35 previously formed sub-base of suitable material, such for example as concrete. After the bricks have been laid on the sand cushion, fluid or plastic material, such as cement, grout or bituminous material is poured in between the brick to secure 40 the same together and to form the separated individual units into one integral layer which constitutes the pavement. It is ordinarily impossible to pour the fluid or plastic material between the brick without pouring an excess amount which 45 spreads over the surface of the brick, and, if bituminous material is employed, renders the same slippery in wet weather.

The surface coating of bitumen is recognized as a serious danger to traffic, and expensive methods have been employed to overcome this danger, the material being some times removed by laborious and expensive scraping methods which are not, however, ordinarily effective, as the upper surfaces of the bricks are not in precisely the 50 same plane, and hence no ordinary scraping oper-

ation is effective to remove all of the material equally over all of the bricks.

My improved invention is effective to provide a brick pavement which is not slippery or dangerous even in wet weather and my method of 60 treatment can be employed either during the construction of the pavement, in which the bitumen has either been carelessly applied over the upper surface of the brick or has expanded and flowed over these surfaces under heat. I 65 will first refer to my improved method of treating an old pavement.

In existing pavements in which the bricks are bonded by bitumen, there are found numerous patches of bitumen which has been spilled onto 70 the upper surface of the bricks or, upon expansion of the bitumen and softening from the heat, has flowed from between the bricks and acted to coat the upper surface. In the treatment of such coating I proceed as illustrated in Fig. 1. 75 There is there shown an ordinary type of brick pavement consisting of a base or foundation 1, a sand cushion 2 superimposed thereon, a series or layer of brick or block 3 mounted upon said sand cushion with the spaces between said blocks 80 filled with a composition 4 of bitumen, which in many cases spreads over the upper surface of the brick or other block in the form of a thin layer 5. In treating this pavement I first apply a layer consisting of a mixture 6 of sand, gaso- 85 line and kerosene in the form of a paste over the coating on the upper surface of the brick. Gasoline and kerosene are then ignited and burned off rapidly, volatilizing some of the oils from the bitumen, and allowing the sand to sink 90 into the bitumen coating and thoroughly impregnate the same, leaving a resulting coating which is a mixture of bitumen and sand, minus any light constituents of the bitumen which have been burned out or volatilized. Following the burn- 95 ing of the gasoline and kerosene, or other material employed, the sand sinks down into the coating 5, producing a new and different type of upper surface 7, which is illustrated in Fig. 2. This new coating offers nearly as good traction 100 as clean brick and there is no danger of vehicles skidding or slipping when passing over a coated pavement which has been so treated.

In the case of a new pavement the treatment is applied at the time of the application of the 105 filler. Ordinarily bitumen, before application in this manner, is heated to about 245° Fahr., at which temperature it is quite liquid, and is then poured between the bricks. In order to treat the bitumen in such a way as to produce a safe pave- 110

ment I preferably heat the bitumen before pouring, to a temperature of about 350° to 400° F. and then add to the fluid material fine, well graded sand or other mineral matter in a considerable quantity. The fluidity of the bitumen allows the sand or other mineral matter to sink in and permeate the entire material, providing an abrasive in the form of sand or other mineral matter in the surface and entirely destroying the slipperiness of the bitumen as ordinarily used. The sand should be added to the bitumen immediately after the latter has been poured in a fluid condition between or on the bricks or other units. The sand should also be heated to a temperature of approximately 400° Fahr., and then applied promptly.

In Fig. 3 I have illustrated the type of pavement just referred to in which the sand-impregnated bitumen extends over the upper surface of the block 3 and into the spaces between these blocks.

In Fig. 4 I have shown a pavement consisting of a concrete base 1, an asphalt surface or covering 8 therefor, the upper portion of the layer 7 of which has been treated in accordance with the method described and has incorporated therein particles of sand or crushed stone to produce a surface having good traction qualities and without the slipperiness when wet of asphalt in its normal condition.

It will of course be understood that in the treatment of old pavements other methods of heating may be employed as a substitute for the application of the gasoline or other combustible material. For example, the surface to be treated may be heated with blow torches or surface heaters or by similar means. Similarly, it will be understood that wherever I have used the word "brick" I employ this term to include pavements formed of brick units proper, or of other units, such as stone or the like, or even pavements which are formed as a whole, such as concrete or asphaltic pavements, in which there is no separation into separate units.

The foregoing method of treating brick pavements has been found to be entirely effective in rendering the surface of bitumen coated spots safe, and it places them in a condition affording the same traction as clean brick. The method is not expensive and can be readily applied as indicated either to old or new pavements.

Other modes of applying the principle of my invention may be employed instead of the one explained, change being made as regards the product and method herein disclosed, provided the step or steps cited by any of the following claims or the equivalent of such be employed.

I therefore particularly point out and distinctly claim as my invention:

1. In a method of treating bitumen coated pavements, the steps which consist in applying a layer of mineral material thereto impregnated with a mixture of combustible material, and then igniting such material to burn the same and melt the bituminous material to permit the incorporation therein of the mineral material.

2. In a method of treating bituminous covered portions of pavement, the steps which consist in first applying to the bituminous coating a layer of mineral material, such material having been moistened with an ignitable liquid which upon burning is capable of producing fluidity in the bituminous coating, then igniting such moistened material and permitting the softening of the bituminous coating and the impregnation thereof by the abrasive material.

3. In a method of treating a bitumen coated pavement, the steps which consist in applying a layer of mineral material thereto impregnated with a mixture of kerosene and gasoline, and then igniting such material to burn the same and melt the bituminous material to permit the incorporation therein of the mineral material.

4. In a method of treating bituminous covered portions of pavement, the steps which consist in first forming a paste of mineral material and ignitable liquid, then applying such paste to said bituminous covered portions and finally igniting such paste, thereby impregnating said bituminous portions with said mineral material to form an abrasive surface.

5. In a method of treating bituminous coated pavements, the steps which consist in applying a paste formed of sand and a combustible liquid to said pavements, and then igniting such paste to burn the same and melt the bituminous material to permit the incorporating therein of said sand.

CARL W. ALLSHOUSE.

55 130

60 135

65 140

70 145

75 150